

# United States Patent Office

2,950,314

Patented Aug. 23, 1960

1

2,950,314

## COLOR COUPLERS FOR COLOR PHOTOGRAPHY

Arthur Henri De Cat, Mortsel-Antwerp, and Raphaël Karel Van Poucke, Mechlin, Belgium, assignors to Gevaert Photo-Producten N.V., Mortsel, Belgium, a Belgian company

No Drawing. Filed Apr. 3, 1956, Ser. No. 575,718

Claims priority, application Great Britain Apr. 5, 1955

2 Claims. (Cl. 260—507)

This invention relates to a process for producing photographic color images by color development, to color couplers for use in such process, and to the preparation of such color couplers.

It is known to produce color photographic images by color development. The color couplers needed for this purpose are preferably incorporated in the photographic emulsion layers or in colloid layers located in the vicinity thereof. In order to prevent wandering of these couplers out of their initial layer into another layer, they are usually loaded by a substituent such as a chain of several carbon atoms. Besides this substituent, other substituents which render the coupler water-soluble are usually introduced. Sulpho groups in particular are effective in this respect.

As couplers for yellow, the acylacetarylides have been used in practice. As acylacetarylides sulphonated in their arylide part, only the acetyl acetarylides have been obtained by allowing diketene to react with sulphonated aniline derivatives. Corresponding sulphonated aroylacetarylides have not been obtained, due to the lack of a suitable method.

An object of the present invention is a method for preparing aroyl-acetylides sulphonated in the arylide part. A further object is a class of new sulphonated aroylacetarylides. Another object is a process for the production of a colored photographic image by the use of these aroyl-acetylides. Still a further object is a light-sensitive photographic material containing such aroyl-acetylides.

Now we have found a method for preparing such aroyl-acetylides sulphonated in the arylide part and it has been found that such compounds are good couplers. In comparison with similar couplers, they are very soluble and are indifferent to silver halide emulsions.

According to the present invention, a reducible silver salt image is developed with a primary amino aromatic developing agent in the presence of an aroyl-acetylide sulphonated in its arylide part wherein the hydrogen atoms of the metehylene group may be replaced by substituents which readily split off on color development.

Further according to the present invention, such compounds are prepared by condensing an aroylacetic ester with a compound of the formula  $\text{NH}_2\text{-aryl-SO}_2\text{F}$ , and by hydrolyzing the resulting sulphonofluoride into the corresponding sulphonic acid or ester. The aryl group of the ester or of the sulphonofluoride may contain a group able to render the coupler fast to diffusion. Alternatively, the aryl group of the ester may contain a nitro group which after condensation may be reduced to an amino group, wherein a group rendering fast to diffusion may be introduced without difficulty.

Compounds of the formula  $\text{NH}_2\text{-aryl-SO}_2\text{F}$  may be obtained in different ways.

Aromatic compounds may be treated with fluorosulphonic acid. Steinkopf (J. prakt. Chem. (2) 117

2

(1927) 1-82) has nitrated two sulphonofluorides, obtained in this way, into

m-Nitro-benzene sulphonofluoride, and  
p-Methyl-m-nitro-benzene sulphonofluoride.

According to W. Davies and J. Dick (J. Chem. Soc. (1931) 2104-09), compounds of the formula

aryl-SO<sub>2</sub>Cl

10 may be treated with potassium fluoride. In this way we have prepared:

o-Nitro-benzene-sulphonofluoride, M.P. 60° C.,  
p-Nitro-benzene-sulphonofluoride, M.P. 80° C.,  
p-Chloro-m-nitro-benzene-sulphonofluoride, M.P. 54° C.,  
and

p - Dimethylamino - m - nitro -benzene -sulphonofluoride,  
M.P. 64° C.

20 The above six nitro-sulphonofluorides have been converted into the corresponding amino compounds by reducing a 25% alcoholic solution of the nitro-sulphonofluoride by means of Raney nickel at 40-100° C. and under a hydrogen pressure of 10-100 atm. After elimination of the Raney nickel, the filtrate is either distilled or evaporated until the amine crystallizes. In this way we have prepared:

m-Amino-benzene-sulphonofluoride, B.P. 160-161° C./14 mm.,

30 o-Amino-benzene-sulphonofluoride, M.P. 62° C.  
p-Amino-benzene-sulphonofluoride, M.P. 68-70° C.,  
p-Chloro-m-amino-benzene-sulphonofluoride, M.P. 69° C.,  
p-Dimethyl-amino-m-amino-benzene-sulphonofluoride, M.P. 58° C.,

35 p-Methyl-m-amino-benzene-sulphonofluoride, M.P. 93° C.

Potassium fluoride may also be allowed to react with acetyl-amino arylene sulphochlorides. The resulting acetylamino-arylene-sulphonofluorides may be de-acylated by means of HCl in alcohol. In this way we have prepared:

p-Methoxy-amino-benzene-sulphonofluoride, M.P. 62° C.,  
2-Methoxy-5-amino-benzene-sulphonofluoride, M.P. 74° C.,  
and

45 2 - 5 - dimethoxy - 3 - amino - benzene - sulphonofluoride,  
M.P. 132° C.

The following reaction exemplifies the production of a sulphonofluoride, fast to diffusion: m-nitro-p-acetyl-amino-benzene-sulphonofluoride, M.P. 122° C., was prepared by slowly adding 22 g. p-acetyl-aminobenzene-sulphonofluoride to a mixture of 68 cm.<sup>3</sup> nitric acid (density 1.48) and 81.5 cm.<sup>3</sup> sulphuric acid (concentrated), pouring the reaction mixture in water, sucking off the precipitate and recrystallizing it from ethyl alcohol. Boiling this acetyl-amino compound in a solution of HCl in methyl alcohol and pouring the mixture in water yields m-nitro-p-amino-benzene-sulphonofluoride, M.P. 148-150° C. By condensing the latter in a known way with

60 CH<sub>3</sub>(CH<sub>2</sub>)<sub>12</sub>COCl  
(myristoyl-chloride), p-myristoyl-amino-m-nitro-benzene-sulphonofluoride, M.P. 64° C. (from acetonitrile), is obtained. Reducing the latter with Raney nickel in dioxane at 40-50° C. and under a hydrogen pressure of 10-50 atm., eliminating the nickel and evaporating the filtrate until the product crystallizes by cooling, yields p-myristoyl-amino-m-amino-benzene-sulphonofluoride, M.P. 122° C.

70 Condensation of these sulphonofluorides with beta-keto esters may be done in the usual way by refluxing the two compounds in toluene or xylene, evaporating the lat-

ter after condensation, and recrystallizing the product. The following compounds were prepared in this way:

m-(p-Hexadecyl-oxy-benzoyl-acetyl-amino)-benzene-sulphofluoride, M.P. 112° C.,  
 p-(p-Hexadecyl-oxy-benzoyl-acetyl - amino)-benzene-sulphofluoride, M.P. 135° C.,  
 p-Methoxy-m-(p-hexadecyl-oxy-benzoyl - acetyl - amino)-benzene-sulphofluoride, M.P. 156° C.,  
 p-Methyl-m-(p-hexadecyl-oxy-benzoyl-acetyl-amino)-benzene-sulphofluoride, M.P. 135° C.,  
 p-(p-Dodecyl-oxy-benzoyl-acetyl-amino)-benzene-sulphofluoride, M.P. 144° C.,  
 m-[p-(p-Isooctyl - phenoxy - ethoxy) - benzoyl] - acetyl-amino-benzene-sulphofluoride, M.P. 148° C.,  
 p-Myristoyl-amino-m-benzoyl-acetyl-amino-benzene - sulphofluoride, M.P. 160° C.,  
 3-(p-hexadecyl-oxy-benzoyl-acetyl - amino) - 6 - methoxy-benzene-sulphofluoride, M.P. 105° C.,  
 3-(p-hexadecyl-oxy-benzoyl-acetyl-amino)-4-chloro-benzene-sulphofluoride, M.P. 132° C.,  
 3-(p-hexadecyl-oxy-benzoyl-acetyl-amino)-4-methyl-benzene-sulphofluoride, M.P. 139° C.,  
 3-(p-hexadecyl-oxy-benzoyl-acetyl-amino)2-5-dimethoxy-benzene-sulphofluoride, M.P. 120° C.,  
 m-(p-Hexadecyl-oxy-naphthoyl-acetyl - amino) - benzene-sulphofluoride, M.P. 98-99° C.,  
 m-(4-Hexadecyl-oxy-3-5-dichloro-benzoyl-acetyl-amino)-benzene-sulphofluoride, M.P. 132-135° C.,  
 m-( $\alpha$ -Hexadecyl-oxy- $\beta$ -naphthoyl-acetyl-amino)-benzene-sulphofluoride, M.P. 90-92° C.,  
 m-(p-Hexadecyl-oxy-m-methoxy-benzoyl-acetyl - amino)-benzene-sulphofluoride, M.P. 97-99° C., and  
 p-(Hexadecyl-oxy-m-methoxy-benzoyl-acetyl-amino)-benzene-sulphofluoride, M.P. 115-116° C.

By condensing m-amino-benzene-sulphofluoride with m-nitro benzoyl-acetic acid ethyl ester and reducing the resulting product with Raney nickel in ethyl alcohol at 60-80° C. and under a hydrogen pressure of 80-100 atm., m-[m-amino-benzoyl-acetyl-amino]-benzene-sulphofluoride was obtained. From the latter were obtained, by condensation with palmitoyl chloride and with alpha-hexa-decyl succinic anhydride:

m-(m-palmitoyl-amino-benzoyl-acetyl - amino) - benzene-sulphofluoride, M.P. 96-98° C., and  
 m-[m(Alpha-hexadecyl-succinyl - amino)benzoyl - acetyl]-benzene-sulphofluoride, M.P. 180° C.

In order to convert the sulphofluorides into the corresponding sulphonic acids, they are first dissolved in acetone or aqueous dioxane and treated at 60° C. with an aqueous solution of sodium hydroxide. After cooling, the sodium salt of the coupler crystallizes out, or is precipitated by the addition of salt. These sodium salts are recrystallized and may easily be dissolved in water or in a mixture of water and alcohol for addition to a silver halide emulsion or to a colloid which will form a layer adjacent to a silver halide emulsion layer or separated therefrom by a water-permeable colloid layer.

As primary aromatic amino developing agents may be used mono-, di- and tri-amino compounds; as mono-amino developers may be mentioned amino phenols and amino cresols, their halogen derivatives, and also amino naphthols.

The developers, which preferably are used and are the most suitable, are the aromatic ortho-, and para-diamines, such as para-phenylene diamine and its substitution products.

5 A photographic film comprising a silver halide emulsion layer or another colloid layer containing a sulphonated aroyl acetylalide according to this invention may be exposed to light, color developed, bleached and fixed in the usual way. In this manner a yellow image is obtained.

10 We claim:

1. Process for the preparation of a sulphonated aroyl acetylalide of the following structure:



15 wherein R represents an aryl radical selected from the group consisting of alkoxyphenyl, alkoxy naphthyl, dialkoxy phenyl, dichloro alkoxy phenyl, isoocetyl phenoxy ethoxy phenyl, nitrophenyl, and acylamino phenyl, R' represents a monocyclic arylene radical of the benzene series, selected from the group consisting of phenylene, chlorophenylene, dialkyl amino phenylene, alkyl phenylene, alkoxy phenylene, dialkoxyphenylene, and acylaminophenylene, and Me represents an alkali metal atom, comprising condensing an aroyl acetic ester of the following formula:



20 30 wherein R'' represents a lower alkyl group, with a compound of the formula  $H_2N-R'-SO_2F$ , and hydrolyzing the resulting compound in the presence of an alkali metal hydroxide.

25 35 2. A sulphonated aroyl-acetylalide of the following structure:



40 wherein R represents an aryl radical selected from the group consisting of alkoxyphenyl, alkoxy naphthyl, dialkoxy phenyl, dichloro alkoxy phenyl, isoocetyl phenoxy ethoxy phenyl, nitrophenyl, and acylamino phenyl, R' represents a monocyclic arylene radical of the benzene series, selected from the group consisting of phenylene, chlorophenylene, dialkyl amino phenylene, alkyl phenylene, alkoxy phenylene, dialkoxyphenylene, and acylaminophenylene, and Me represents an alkali metal atom, said sulphonated aroyl acetylalide being prepared by condensing an aroyl acetic ester of the following formula:



45 50 wherein R'' represents a lower alkyl group, with a compound of the formula  $H_2N-R'-SO_2F$ , and hydrolyzing the resulting compound in the presence of an alkali metal hydroxide.

#### References Cited in the file of this patent

#### UNITED STATES PATENTS

|    |           |                        |               |
|----|-----------|------------------------|---------------|
| 60 | 1,971,409 | Henle et al. -----     | Aug. 28, 1934 |
|    | 2,083,962 | Petitcolas -----       | June 15, 1937 |
|    | 2,303,928 | Froehlick et al. ----- | Dec. 1, 1942  |
|    | 2,312,040 | Kendall et al. -----   | Feb. 23, 1943 |
|    | 2,748,164 | Dodson -----           | May 29, 1956  |